

Oct. 24, 1944.

C. A. JENSEN

2,361,106

METHOD OF REPAIRING AND FOR PREVENTING CRACKS IN METAL CASTINGS

Filed Nov. 4, 1940



INVENTOR:  
CHARLES A. JENSEN.  
By Morten O. Smith, ATTY.

## UNITED STATES PATENT OFFICE

2,361,106

## METHOD OF REPAIRING AND FOR PREVENTING CRACKS IN METAL CASTINGS

Charles A. Jensen, Inglewood, Calif.

Application November 4, 1940, Serial No. 364,204

3 Claims. (Cl. 29—148)

My invention relates to a method of repairing cracks in metal castings and for preventing cracks that may develop in castings and particularly weakened portions thereof or portions that are subject to extreme variations of temperature, for instance, the cylinder blocks and heads of internal combustion engines, Diesel engine heads, and the like, and the methods herein disclosed are an improvement on the method of repairing cracks in metal castings patented by me February 5, 1935, Patent No. 1,989,695.

The principal objects of my invention are to generally improve upon and simplify the method disclosed in my aforesaid patent, as well as other similar methods, and further, to provide a relatively simple and easily practiced method of repairing cracks in metal castings and for preventing the development of cracks in metal castings, which method involves the following essential steps, namely, the closing of the crack in a casting by the use of tie rods or bolts, the drilling of holes along or adjacent the crack, the insertion of a sealing material in the cracks and holes, the insertion of tapered pins or plugs into the drill holes, the inner portions of which pins extend into the cooling fluid circulation chamber or chambers within the casting by peening the metal along or adjacent the edges of the crack or by connecting the edges of the crack by brazing or welding.

My invention contemplates the practicing of any one, two, or more of the steps just set forth and further, any one, two, or more steps of the method may be utilized for preventing the development of cracks in weak portions of metal castings or portions that are subjected to extreme variations of temperature, for instance, the metal adjacent the exhaust ports of internal combustion engines or the thick sections of metal between the ports of Diesel engine heads.

In the accompanying drawing:

Fig. 1 is a top plan view of an internal combustion engine cylinder block that is reinforced with transversely disposed tie bolts and showing cracks that have been repaired in accordance with my improved method.

Fig. 2 is an enlarged vertical section taken on the line 2—2 of Fig. 1.

Fig. 3 is a plan view of a portion of a cylinder block and showing a crack between a valve port and circulation opening repaired in accordance with my improved method.

Fig. 4 is a vertical section taken on the line 4—4 of Fig. 3.

Fig. 5 is a detail plan view of a portion of a

cylinder block with arrows indicating the approximate position of the lines of force in a shrunken portion of the block between the piston chamber and exhaust valve port and which portion is generally referred to as a "hot spot" due to the extremely high temperatures developed by the exhaust gases in passing from the piston chamber to the exhaust port.

Fig. 6 is a plan view similar to Fig. 5 and showing the metal in the "hot spot" expanded by an inserted pin or plug so as to materially strengthen the metal in this particular portion of the casting and counteract tendency to crack.

Fig. 7 is a plan view of a portion of a casting 15 having a crack that has been repaired in accordance with my improved method and the metal beyond the ends of the crack having been acted upon so as to effectively counteract tendency to increase in length.

Fig. 8 is a plan view of a portion of a cylinder block having a crack closed and sealed in accordance with my method and through the use of a single pin or plug.

Fig. 9 is a cross section taken on the line 9—9 of Fig. 8.

Fig. 10 is an elevational view of a portion of a Diesel engine head and showing a crack therein repaired in accordance with my improved method.

Fig. 11 is an enlarged cross section taken on the line 11—11 of Fig. 10.

Referring by numerals to the accompanying drawing and particularly to the construction illustrated in Figs. 1 and 2, 10 designates the cylinder block of an internal combustion engine having the usual piston chambers 11, exhaust valve ports 12, inlet valve ports 13, and circulation fluid openings 14 that communicate with the circulation chambers in the block around the cylinders and the ports. Cracks C1 are shown in the block between the piston chambers 11 and one of the water passages 14, a crack C2 between one of the exhaust ports 12 and one of the water passages 14, and a crack C3 between one of the piston chambers and one of the exhaust ports.

Where the cracks extend substantially lengthwise of the cylinder block, the latter is put under a certain degree of compression transversely by means of tie bolts 15 that pass transversely through the block just beneath the top thereof, the heads of said bolts being preferably countersunk and their threaded ends being provided with nuts 16. These nuts are tightened to place the block under transverse compression strains in order to resist tendency of the cracks in the block to increase in length during a subsequent

step in the method. By placing proper tension on the tie bolts, the cracks in the casting may be practically closed.

Tapered holes are now drilled in the casting along the cracks after which a suitable sealing compound, either metal or cement, is now driven or calked into the cracks and into the holes drilled therein.

Tapered pins or plugs 17 are now driven into the tapered holes so as to expel the sealing compound therefrom and force the same into the cracks adjacent the plugs, thereby compressing said sealing compound and likewise placing the adjacent metal under compression strains. The compression strains produced by driving the tapered pins into the casting are counter-opposed to the compression strains produced by the bolts 15 and nuts 16, and thus the solidity of the metal in the casting immediately adjacent the crack is greatly increased. The tapered pins or plugs may be threaded and screwed into the holes in the block and in order to enhance the cooling effect of the water or other cooling fluid that is circulated through the chambers in the block surrounding the piston chambers and ports, the length of the inserted pins or plugs is such that their inner portions extend substantial distances into the cooling fluid circulation chambers as illustrated in Fig. 2.

The metal in the casting adjacent the cracks and inserted pins is now brought together by being peened with a hammer or like tool or by brazing or welding the edges of the metal to each other along the cracks.

In practicing my improved method as just described, the tie bolts are utilized to close and maintain the cracks in closed position before the tapered pins, plugs or wedges, are inserted, thereby enabling greater wedging pressure to be impressed on the adjacent metal so as to solidify said metal throughout the cracked area and consequently insuring a perfect seal after the work incident to the practicing of the method has been accomplished.

In Figs. 3 and 4 I have illustrated a crack between an exhaust valve and a water passage sealed by means of a single tapered pin or plug and with the sealing compound driven into the crack under compression, and in Fig. 3 arrow heads show the direction of the lines of compression developed by the driving of the pin into the casting, thus solidifying the entire area of metal between the openings and providing an effective seal.

Thus the wedging action of the inserted pin or plug reverses the lines of force in the casting, particularly if the crack occurs in a "hot spot" or an area that is subjected to a wide range of temperatures and such practice is very effective in both old and new engines regardless of whether they are cracked or not.

In Fig. 5 I have illustrated a portion of a cylinder block having a piston chamber 18 and an exhaust port 19, with an intervening "hot spot" or area that is subjected to extreme temperatures, with arrow heads showing the approximate position of the lines of force in the metal throughout the "hot spot" area and adjacent metal.

To fortify and materially increase the resistance to cracking in this "hot spot" area, a tapered pin or plug such as 20 is driven into a tapered hole formed in the metal between the chamber 18 and port 19 with sufficient wedging action to reverse the lines of force in that portion of the metal in the "hot spot" so that such lines of force take the

approximate position as indicated by the arrow heads in Fig. 6.

In cylinder blocks "hot spots" develop near exhaust ports for the reason that the surrounding metal is very much cooler while the engine is in operation. The air and water cooled outer surface functions as a tight band around the "spot" and as the colder metal has greater strength and stability, the "hot spot" will be compressed due to the fact that the metal when heated becomes somewhat softer. The "hot spot" remains compressed after the engine ceases to operate and has become cool. The compressed "spot" now occupies a smaller area which develops pulling strains between it and the surrounding area. Continued starting and stopping of the engine increases these strains until the metal parts or cracks and such condition is very frequently found in old engines between the valve ports or between the valve ports and the piston chambers.

Thus my improved method can be carried out at the point where these cracks are liable to develop and consequently the method is particularly effective and has the added advantage of preventing cracks in metal castings at the points where cracks are liable to occur.

The driving of a round wedge such as a tapered pin into the tapered hole in the "hot spot" of a cylinder block causes compression of the metal immediately adjacent the wedge and the development of outward or pushing strains of the metal within the "hot spot" is produced.

It is to be noted that this condition is exactly opposite that found in an engine after it has been in use and it will also be noted that if this condition is created in a new engine cylinder block, it will materially increase its life or period of usefulness.

"Hot spots" generally develop adjacent exhaust valve seats with the resulting action of swelling or expanding one side of the seat, which prevents proper seating of the valve and reduces compression. "Hot spots" also cause shrinkage of the adjacent cylinder wall.

By my improved method, the temperature changes in the "hot spot" are materially reduced by extending the tapered pins, plugs or wedges, into the cooling medium that circulates through the block, thus counteracting tendency of the valve seat to swell on one side and shrinkage of the adjacent cylinder wall, with the result that compression in the cylinder is materially increased.

Cracks in the "hot spots" of castings are usually increased slightly in length when the wedges are driven into the holes. However, this is beneficial due to the removal of the pulling strains still in the metal immediately adjacent the crack or fracture. The crack is finally sealed by placing sealing material therein or by drawing its edges together by peening or calking.

In the event that it becomes necessary to prevent parallel movement of the metal adjacent the crack, a threaded tapered pin or plug in a threaded tapered hole is utilized to create the necessary pressure and after such pressure is developed, a solid row of pipe plugs may be used or sealing material may be calked into the crack where the metal is very thin.

Under certain conditions all three sealing means, namely, the insertion of tapered pins, the use of a sealing compound, and peening of metal adjacent the crack, may be used and flat or other shaped wedges may be used to change the direc-

tion of the pressure in the metal adjacent the crack when necessary.

In Fig. 7 I have illustrated the treatment of a crack in accordance with my invention for preventing said crack from lengthening and practically the same treatment may be utilized for preventing the development of cracks in new castings. Where a crack in a casting exists, tapered holes are drilled along the crack and tapered pins or plugs such as 21 are driven into said holes so as to compress and thereby strengthen the metal adjacent the crack and which action may slightly widen the crack particularly at the ends thereof.

In some instances it may be found desirable to bore the tapered pin or plug receiving holes in the casting near the ends of the crack to the sides thereof.

The second step in this method is to remove the tension and tendency in the metal to pull apart near the ends of the crack so as to prevent extension thereof and this is done by compressing or peening the metal beyond the ends of the crack, the areas of such compression or peening being substantially V-shape with the wide portions thereof disposed adjacent the ends of the crack so as to taper off the strains impressed in the metal outwardly from the crack. Finally the crack is closed by the insertion of a sealing compound and the peening of the edges of the metal immediately adjacent the crack or by brazing or welding.

Obviously, the method just described may be utilized for preventing cracks in new castings at points or areas where the development of cracks might be expected.

A variation of the method just described would be to first peen the metal beyond the ends of the crack and afterwards drill the holes along or adjacent the crack for the reception of the tapered pins or plugs.

Where my improved method is utilized for preventing cracks in metal castings, the casting strains developed by a "hot spot" are reversed and the inserted pins that extend into the cooling fluid circulation chambers are highly effective in absorbing the heat normally existing in the "hot spots" and spreading opposite tension around the "spot" and which advantageous result is enhanced by the peening or hammering of the metal adjacent the crack or "hot spot."

Thus my improved method involves the development of an excessive amount of pressure or more than is required to prevent the development of a crack and a highly beneficial force is stored in castings and which force may be and is drawn on as the engine is operated.

Thus the parting or cracking of the metal in the treated areas is not likely as long as the force installed remains in the metal and such force may be renewed by the insertion of new pins in the casting.

In Figs. 8 and 9 I have illustrated the sealing of a superficial crack with a single inserted wedge-like member, for instance, a tapered pin or plug, and where such practice is carried out a tapered hole is bored in the metal so that it intersects the crack and a single pin such as 22 is driven into said hole, with the inner portion of said pin projecting into the cooling fluid circulation chamber.

Thus a portion of the inserted pin is seated in a solid portion of the casting with another portion of the pin completely sealing the crack and which result is attained without the use of seal-

ing material and without peening or brazing the metal along the edges of the crack.

In Figs. 10 and 11 I have illustrated the repair of a Diesel engine head in accordance with my invention.

The thick sections between the ports of Diesel engine heads become extremely hot due to the extremely high compression and the cooling effect of the circulation fluid is reduced on account of its being so far from the combustion chamber due to the great thickness of the metal. Under such conditions cracks form, generally between the valve chamber 23 and the injector port 24. A hole 25 is drilled into the metal between the chamber 23 and injector port 24, which hole intersects the crack and a pin or plug 26 is driven into said hole so as to effectively stop the gas leak between the port and valve chamber. Inclined holes 27 are now bored in the head from a point directly above the hole 25 and pin 26 and which holes 27 diverge toward their lower ends.

The formation of these holes removes the upper end portion of the inserted pin 26 so that the upper end thereof is wedge-shape in cross section. A pin 28 is driven into one of the inclined holes 27 so that its upper end is slightly below the surface of the metal in which the holes are bored and a third pin 29 is now driven into the other one of the holes 27, with the upper end of said third pin lying flush with the outer surface of the engine head. Thus the upper ends of all three pins are in direct contact with each other.

Inasmuch as the inclined pins 28 and 29 extend substantial distances into the cooling fluid circulation chamber in the head, the cooling effect of the circulating medium is transferred to the upper portion of pin 26 and to the external surface of that portion of the head in which the crack is located so as to bring about maximum cooling effects to counteract tendency of warping of the valve seat and at the same time stopping leakage of gas.

Large and heavy castings, for instance, internal combustion engine cylinder blocks and Diesel engine heads frequently shrink at various points when cooling off after casting and which shrinking action develops internal casting strains and by using the power of the wedge in the areas having these internal strains, the latter are relieved with the result that the life or periods of usefulness of the treated castings are materially increased.

Thus it will be seen that I have provided a relatively simple and easily practiced method for repairing cracks in metal castings and which method may be used with equal advantage in preventing the development of cracks in castings by the strengthening and reinforcement of those parts of the castings where cracks are liable to develop.

I claim as my invention:

1. The method of repairing cracks in metal castings which consists in placing the casting under compression strains applied to said casting at points on opposite sides of the crack therein, so that the lines of compressive forces are directed from both sides toward said casting crack compressing the metal in the casting beyond the ends of said crack, the areas of which compression taper away from said crack in approximate longitudinal alignment therewith, then forming holes in said casting along the crack therein, then filling said holes with a sealing compound, then applying pressure to said sealing compound so as to force same into those portions of the crack

between said holes and then uniting the edges of the crack along the surface of the casting so as to confine the compressed sealing compound within said crack.

2. The method of repairing cracks in metal castings which consists in placing the casting under compression strains applied to said casting at points on opposite sides of the crack therein, so that the lines of compressive force are directed from both sides toward the crack compressing substantially triangular areas of metal in casting beyond the ends of said crack, with the bases of said triangular areas disposed substantially at right angles to the linear position of said crack, then forming holes in said casting along the crack 15

therein, then filling said holes with a sealing compound and driving tapered pins into said holes to force and compress the sealing compound therefrom into those portions of the crack between said holes and at the same time compressing and solidifying the metal in the casting adjacent said holes.

3. The method of repairing metal cracks in metal castings as set forth in claim 2 and then connecting the edges of the surface of the metal throughout the length of the crack so as to confine the compressed sealing compound within said crack.

CHARLES A. JENSEN.